

[54] MELTING AND CASTING OF  
TRANSITIONAL METALS AND ALLOYS

[75] Inventors: **Kenneth Aldersley**, Reading;  
**Gordon William Telford**, Tadley,  
both of England

[73] Assignee: **United Kingdom Atomic Energy  
Authority**, London, England

[22] Filed: **May 18, 1973**

[21] Appl. No.: **361,490**

[30] Foreign Application Priority Data

May 23, 1972 Great Britain..... 24184/72

[52] U.S. Cl. .... **75/10 R, 75/65 R**

[51] Int. Cl. .... **C22d 7/04**

[58] Field of Search ..... 75/10, 84; 164/80, 51

[56] References Cited

UNITED STATES PATENTS

3,264,093 8/1966 Sump ..... 75/10 R

|           |         |              |         |
|-----------|---------|--------------|---------|
| 3,484,840 | 12/1969 | Spoth.....   | 164/80  |
| 3,504,093 | 3/1970  | Persson..... | 75/10 R |
| 3,598,168 | 8/1971  | Clark.....   | 164/51  |

Primary Examiner—L. DeWayne Rutledge

Assistant Examiner—Peter D. Rosenberg

Attorney, Agent, or Firm—Larson, Taylor and Hinds

[57] ABSTRACT

A method of melting and casting a transitional metal or an alloy thereof uses an unclad thin-walled graphite crucible having a bottom opening therein in which is positioned a fusible metallic member, usually alike the charge metal in composition, to obturate the opening; charge metal is positioned in the crucible and is rapidly heated by electrical induction to a temperature above its melting temperature without substantially melting the obturating member, and thereby provides a pool of molten metal flowing onto the member to melt a pour hole therethrough through which the molten charge discharges from the crucible.

10 Claims, 1 Drawing Figure



PATENTED DEC 31 1974

3,857,696



## MELTING AND CASTING OF TRANSITIONAL METALS AND ALLOYS

### BACKGROUND OF THE INVENTION

This invention relates to the melting and casting of transitional metals and alloys thereof having high melting temperatures and, in particular, to the melting and casting of titanium and titanium alloys.

U.S. Pat. No. 3,484,840 discloses a method of melting titanium alloys which comprises providing a refractory ceramic crucible having a bottom opening therein, positioning an electrically conductive graphite sleeve within said crucible, positioning a titanium alloy disc at the base of the sleeve and extending completely across said bottom opening, positioning a charge of the alloy to be melted within said sleeve and in spaced relation to said disc, and rapidly inductively heating such charge above its melting point without similarly melting the disc, to thereby provide a pool of molten metal flowing onto the disc and thereby melt an opening through the disc.

The specification explains the disadvantages of skull melting in water-cooled crucible arc-melting units, namely the need for specialized and high cost equipment, the difficulty in achieving temperature control whence the variation in pouring temperatures can cause casting defects and the hazard of arc-melting using water-cooled crucibles. The specification states that the above-cited method utilises equipment which can be installed and operated by investment casting foundries without substantial capital expenditure, that the method provides a much better control of the pouring temperature and that the cost of melting and pouring titanium, using the method, is significantly reduced.

It has now been unexpectedly established that a container vessel in the form of a refractory ceramic crucible is unnecessary in the melting of titanium and its alloys and that a graphite crucible thin enough for the inductive power loss therein to be low is capable of holding the molten charge without bursting, even though not supported within a ceramic casing.

Accordingly it is an object of the present invention to provide an improved inductive heating method for melting and casting titanium and other transitional metals and the alloys thereof having high melting temperatures.

### SUMMARY OF THE INVENTION

According to the invention a method of melting and casting a transitional metal or an alloy thereof comprises providing an unclad thin-walled graphite crucible having a bottom opening therein, positioning a fusible metallic member substantially non-deleterious to the molten charge metal at the bottom of said crucible to obturate said opening, positioning a charge of said metal or alloy to be melted within said crucible above said member and rapidly heating said charge by electrical induction to a temperature above its melting temperature without substantially melting said member to thereby provide a pool of molten metal flowing onto the member and thereby melt a pour hole through the member through which the molten charge discharges from the crucible.

The graphite crucible may have a wall thickness substantially less than the electrical reference depth  $\alpha$  where  $\alpha = (1/2 \pi) \nu (\rho/\mu f)$   $\rho$  being the resistivity of

graphite (1300 microhm/cm),  $\mu$  the permeability of graphite (1, for a non-ferrous material) and  $f$  the frequency of the electrical supply. In practice, it is found that the wall thickness may be less than one-fifth the electrical reference depth and preferably is less than one-tenth.

The crucible wall should have a thickness such that the crucible is mechanically strong enough to hold the charge metal yet be such that energy generated by the induction coil is absorbed mainly in the metal charge to be melted, graphite being, electrically, a susceptor material.

The molten charge metal exerts its maximum lateral thrust at a position close to the bottom of the crucible; to provide support for the crucible in this region it is preferred to seat the crucible in a refractory supporting cup the walls of which form a sliding fit with said crucible and extend to embrace the crucible over said region, said cup having a bottom opening enabling molten charge metal to flow from the crucible. Preferably the supporting cup is made of graphite thereby functioning as a heat sink for heat transmitted through the lower wall of the crucible.

To reduce carbon pick-up by the molten metal from the crucible wall the crucible may be lined with a ceramic material subsequently inert to the molten metal. Suitable materials for use with titanium and titanium alloys include tungsten, yttria-stabilised zirconia, and yttria- or calcium-stabilised zirconia mixed with titanium hydride. The material may be present as a coating applied by plasma spraying. Alternatively, free-standing liners fabricated from these materials may be inserted into the crucible to be in contact with and to protect the crucible wall.

The fusible metallic member may be made from said metal or an alloy thereof.

Transitional metals reactive to air in the molten state, such as Ti and its alloys, are preferably inductively heated in vacuo.

The invention also provides apparatus for melting and casting a transitional metal or an alloy thereof comprising an unclad thin-walled graphite crucible having an opening in the base thereof for the discharge of molten charge metal there-through, and in which a fusible metallic member is locatable to obturate the opening, and an electrical inductor heating coil disposed without said crucible and locatable in relation thereto such that a charge of said metal or alloy, containable within the crucible above said obturating member, is within the field of said coil.

The fusible metallic member may be made from metal or an alloy thereof.

The inductor heating coil may include, in addition to a plurality of coil turns providing the magnetic flux for melting, at least one reverse wound turn so spaced from said plurality of turns to be positionable in relation to the rim of the crucible to substantially curtain metal splash-over during meltdown.

By the use of electric induction heating rather than heating by an electric arc the stirring effect in the molten metal produced by induction heating ensures that, immediately prior to the melting of the metallic member, the whole of the molten charge is at a substantially uniform temperature. As a result of this stirring action the whole of a molten charge, immediately prior to casting, can not only be raised to a uniform temperature for efficient casting but can also be made to dis-

charge from the crucible at a substantially constant temperature in successive melts. A temperature variation of about 25°C in the casting temperature, in successive melts, has been found possible.

#### DESCRIPTION OF THE DRAWING

The nature of the present invention is hereafter further explained, by way of example, with reference to the accompanying drawing illustrating a sectional elevation of one melting and casting apparatus.

The melting and casting apparatus shown is approximately to scale and has an unclad thin-walled graphite crucible 1 located within an inductor coil 2. The crucible is supported by a shallow cup 3 provided with support legs 4. The cup 3 has a bottom opening 12 within which is located a spout 11 supported by shoulders at its uppermost end. The lower part of the crucible is a sliding fit within the walls of the cup: when a charge of metal 6 is rendered molten by high rate inductive heating the molten charge exerts its maximum lateral thrust against the supporting crucible a short distance from the bottom of the crucible; at greater distances from the bottom the metal tends to retract inwards from the crucible wall. The cup 3 provides lateral support for the crucible over this short distance from the bottom and being made of graphite also acts as a localised heat sink. To curtain susception in the cup wall 5 three vertical slots are cut through the wall (not shown) the slots being cut at intervals of 120°: one slot is extended to cut through the base of the cup and forms a radial slot therein; this has been sufficient to curtain susception in the base.

The crucible 1 has an opening 7 in its base 8 for the discharge of the molten charge from the crucible. The opening 7 is obturated by a metallic member 9 which, in this embodiment, is in the form of a stepped plug seated in the opening. The plug 9 is surrounded by an annular insert 10 made of graphite: the insert is slotted through vertically (slot not shown) to curtain susception and provides a false bottom with the plug 9 positioned centrally therein. The spout 11 is also made of graphite. It will be apparent that the crucible 1 serves to short-circuit the slots cut through the cup wall 5: to obviate this effect thin coatings of alumina are painted or sprayed on the inside of the cup wall and/or on the outside of the crucible where it slides into the cup.

The inductor coil 12 has 14 turns and, spaced above the crucible, 2 reverse wound turns 13. The reverse wound turns create a magnetic field in opposition to that created by the lower 14 turns and serve to curtain metal splash-over which can otherwise occur when HF power for high rate heating is applied to the coil 2. The reverse wound turns thus allow the requisite power to be applied without causing an unstable melt.

#### EXAMPLES OF THE PRESENT PROCESS

The apparatus of the present embodiment has been used for melting Ti and Ti alloys. Short bars of metal 2½ ins dia × 3 ins were inserted into the 2.6 in dia crucible to rest on the false bottom 10, as shown.

The electrical measurements for a typical melt were

as follows - (the charge metal was 90% Ti 6% Al 4% alloy)

Inductance of 14 turn coil = 10.85  $\mu$ H

| 5       | Capacity in Circuit KVA | Alternator Volts | Alternator Amps | KW | KVAR | Field Current (amps) |
|---------|-------------------------|------------------|-----------------|----|------|----------------------|
| 10      | Empty coil              | 360.0            | 350             | 75 | 26   | -7                   |
| To Melt | 380.0                   | 350              | 146             | 50 | -8   | 1.90<br>2.15         |

The wall thickness of the crucible 1 was within the range 0.050–0.070 ins and the base thickness also in the range 0.050–0.070 ins. By using a crucible having these dimensions the crucible is "electrically and mechanically thin;" a large proportion of the electrical power is absorbed by the charge. Moreover, a thin crucible can better i) withstand the thermal shock due to the rapid heat rate developed when power is applied and ii) promote a high rate of heat loss by radiation thus effectively cooling the inner crucible surface. If the inner crucible surface can be kept "chilled" by high radiant heat loss, the rate of reaction between the crucible and a melt can be substantially reduced.

Thus the requirements for a crucible as used in the present invention are i) a capability to hold the charge ii) low power consumption and iii) high radiant heat loss. It will be apparent that the need for a crucible of sufficient strength to hold the charge is the limiting factor.

In practising the present invention high heating rates and short heat times are preferably used to reduce carbon pick-up. Carbon pick-up can be further reduced by lining, or providing liners for, the inner surface of the crucible. The crucible can be lined with (for Ti and Ti alloys) tungsten, yttria-stabilised zirconia, or yttria- or calcium-stabilised zirconia with titanium hydride, and these materials can be applied by plasma spraying: alternatively free-standing liners in these materials can be produced by plasma spraying and the liners slipped inside the crucible.

Crucibles for use in the present invention can be made, for example, by i) machining from dense graphite masses, ii) machining from porous graphite and densifying the inner surface with pyrolytic graphite to impede metal penetration and confer additional strength, iii) deposition of pyrolytic graphite onto a mandrel and iv) spraying graphite into carbon fibre or cloth wound on a mandrel and consolidating the inner surface of the crucible so formed with pyrolytic graphite. Lined crucibles can be made by deposition of liner material onto a mandrel followed by a graphite backing produced by, for example, spraying or by deposition of pyrolytic graphite.

For apparatus of larger size than that of the embodiment to wall thickness of the crucible may be increased within limits: to retain low power absorption with thicker-walled crucibles the frequency of the HF power supply has to be lowered.

The following Table collates heat times with the carbon content and hardness values for charge metal and cast metal when melted in unlined and lined crucibles. The charge metal was a Ti alloy (90% Ti 6% Al 4% V).

| Crucible Structure                                                      | Heat Time Mins | Carbon Content % |             | Hardness, VPN |            |
|-------------------------------------------------------------------------|----------------|------------------|-------------|---------------|------------|
|                                                                         |                | Charge metal     | cast metal  | Charge metal  | cast metal |
| Dense Graphite Graphite (20-30% porosity) lined with Pyrolytic graphite | 2.05           | 0.045            | 0.230       | 330           | 345-380    |
|                                                                         | 2.00           | 0.045            | 0.089-0.22  | 330           | 345-376    |
| Dense graphite Liner: Yttria stab. Zirconia                             | 2.00           | 0.045            | 0.040-0.048 | 330           | 272.363    |
| Dense Graphite Liner: Yttria stab. Zirconia                             | 2.50           | 0.045            | 0.042-0.060 | 330           | 309-350    |
| Dense Graphite Liner: yttria stab. Zirconia + Ti                        | 2.40           | 0.045            | 0.042-0.067 | 330           | 300-355    |

In melting Ti and Ti alloys the apparatus of the present invention is held in vacuo: U.S. Pat. No. 3,484,840 draws attention to the problem of contamination in the melting and casting of titanium and mentions the embrittling effect of hydrogen, oxygen, carbon and nitrogen; accordingly air should be excluded from the melt environment so far as is practicable.

Although the above embodiment of the invention is concerned with titanium and its alloys the invention has application to high-melting transitional metals in general. Uranium and uranium alloys can, for example, with advantage be melted and cast according to the invention. It is believed that, like Ti, the reactive nature of many of these metals when molten is curtailed by the high radiant heat loss from the thin-walled crucibles of the invention and that by inducing "chill" at the metal-crucible interface in this manner the rate of reaction in the region of this interface is substantially reduced: lined or unlined crucibles can be used according to the reactive habit of individual metals.

What we claim is:

1. A method of melting and pouring as a molten charge a transitional metal or an alloy thereof comprising providing an unclad, thin-walled graphite crucible having a bottom opening therein, positioning a fusible metallic member substantially non-deleterious to the molten charge metal at the bottom of said crucible to obturate said opening, positioning a charge of said metal or alloy to be melted within said crucible above said member and rapidly heating said charge by electrical induction to a temperature above its melting temperature without substantially melting said member to thereby provide a pool of molten metal flowing onto the member and thereby melt a pour hole through the member through which the molten charge discharges from the crucible.

2. A method as claimed in claim 1 wherein the graphite crucible has a wall thickness substantially less than the electrical reference depth,  $\alpha$ , as herein before defined.

3. A method as claimed in claim 2 wherein the crucible wall thickness is less than one-fifth the electrical reference depth.

4. A method as claimed in claim 3 wherein the crucible wall thickness is less than one-tenth the electrical reference depth.

5. A method as claimed in claim 2 including seating the crucible in a refractory supporting cup the inner wall of which forms a slidable fit with the crucible outer wall and extends to embrace the lower region of the crucible.

6. A method as claimed in claim 5 in which the supporting cup is a graphite cup.

7. A method as claimed in claim 5 wherein the inner wall of the crucible is lined with a ceramic material substantially inert to the molten metal.

8. A method as claimed in claim 7 wherein, in the melting of Ti and Ti alloys, the ceramic material is chosen from tungsten, yttria-stabilised zirconia and yttria- or calcium-stabilised zirconia mixed with titanium hydride.

9. A method as claimed in claim 7 wherein the crucible lining is provided by plasma spraying a coating of the ceramic material onto the inner wall of the crucible.

10. A method as claimed in claim 7 wherein the crucible lining is provided by inserting a free-standing liner, fabricated from the ceramic material, into the crucible.

\* \* \* \* \*